

## UNITED STATES PATENT OFFICE

2,145,989

## METHOD OF TREATING METALS

William J. Merten, Pittsburgh, Pa., assignor to  
 Bocjl Corporation, Pittsburgh, Pa., a corpora-  
 tion of Delaware

No Drawing. Application June 18, 1937,  
 Serial No. 148,955

10 Claims. (Cl. 148—12)

This invention relates to a method of treating steel to produce articles, especially springs and the like, possessing particularly desirable mechanical properties.

5 It is among the objects of the invention to provide a method of treating steel which confers a combination of properties of a particularly desirable character, especially for the production of helical and elliptical springs, which eliminates the necessity for cold-working while providing satisfactory hardness, strength and other mechanical properties, is cheap and easily practiced, and provides a grain structure in the finished article that is particularly suited to the requirements of 10 springs.

A particular object is to provide steel articles possessing a fibrous structure comprising elongated grains disposed parallel to the main axis of the article, and which in the hardened condition 15 embody highly desirable mechanical properties.

The invention is predicated upon my discovery that its stated objects are attained by hot-working a piece of steel to form stock which is oversized relative to the final product, then sizing the stock to bring it to the dimensions of the finished article by working it hot but at a temperature below the recrystallization range, to thereby produce a hot-sized shape having a fibrous structure composed of elongate parallel grains disposed in alignment with the longitudinal axis of the shape. 20 The sized article thus produced by hot-working is then subjected to a hardening operation without destruction of the fibrous structure which characterizes the product of the invention. This is accomplished by heating the article rapidly to a temperature within the austenite range, followed by quenching, both steps being so conducted as to effect the desired hardening while preserving the fibrous structure substantially without change. Following this the heat-treated article may be 25 tempered if desired.

Thus it will be seen that it is of the gist of this invention that by hot-working there is produced an article which is sized and possesses a fibrous structure in which the fibers lie in the direction 30 of working, and such structure is preserved in subsequent heat treatment for hardening.

The manner of conducting the hardening step constitutes an important feature of the invention because it must be so conducted as to effect hardening without material destruction of the fibrous structure. To this end the article is brought rapidly into the austenite temperature range, and the quenching is carried out quickly to preserve the grain size and fibrous structure of the article. Stated otherwise, in the practice of the invention the conversion of the fibrous grains to equi-axed grains is avoided as far as possible so that the hardening step is effected in such manner as 35 substantially to avoid recrystallization and thus

with substantial preservation of the fibrous structure.

If the heating step of the hardening operation is carried out properly, the recrystallization will proceed only incipiently, and provided it does not proceed so far as to substantially alter the fibrous structure, such incipient recrystallization is desirable because apparently it produces an interlocking of the fibers with consequent increase in the cohesive forces between them, which increases the 10 strength of the product.

When the article has been heated sufficiently, i. e., when the heat has penetrated the article, it is quenched with sufficient rapidity to avoid recrystallization to any substantial extent. Provided it be done rapidly, the article may be formed between the heating and quenching stages of the heat treatment. After quenching, the article may be tempered, or drawn, as need be.

Although not restricted thereto, the invention is especially adapted to the manufacture of 20 springs or stock for making springs, for which reason it may be described with particular reference thereto, elliptical springs being chosen by way of example. In the practice of such an embodiment of the invention a billet or ingot of 25 steel of suitable composition is hot-rolled in accordance with standard practice except that whereas it is customary in the manufacture of elliptical springs to hot-roll (i. e., at temperatures productive of recrystallization) down to the 30 finished size of the spring leaves, in accordance with the present invention there is produced by hot-working stock, such as strip or rod, which is oversized, i. e., whose cross-sectional area is 35 greater than that of the finished leaf. This oversized stock is then subjected to hot-finishing at a temperature slightly below the recrystallization range of the steel, i. e., at a temperature below that used in true hot-working. Ordinarily it is 40 possible to so correlate the temperature of the ingot or billet and the hot-rolling to the oversized shape that the shape will then be at a suitable temperature for the finishing pass, but if necessary or desirable for any reason the oversized stock may be reheated until it is at a temperature 45 appropriate for the hot-finishing pass (below the recrystallization temperature).

As is characteristic of products made in accordance with this invention, the hot-sized shape is provided with a fibrous grain structure in which the grains are elongated in the direction of working so that they are parallel and are aligned with the longitudinal axis of the shape. Such a structure is highly desirable for many purposes, and through it there is attained, after appropriate hardening, a highly desirable combination of 50 mechanical and physical properties.

In the practice of the invention as applied to 55 the production of elliptical springs, the hot-sized

60

shape is cut to lengths appropriate for the manufacture of spring leaves. These are then heated rapidly, as described above, in a suitable medium, such as a fused salt bath, a mixture of equal parts of sodium and potassium chlorides affording a bath suitable for many purposes. The bath is heated to a temperature such that the article will be brought rapidly to the desired temperature, the mass of the bath being such that its temperature will not be materially decreased in consequence of the introduction of the piece.

When the heat has penetrated the piece sufficiently it is removed, placed in the forming dies, pressed quickly to shape, and immediately quenched, suitably while still held in the dies, precautions being taken to insure that the quenching is sufficiently rapid to produce maximum hardness and also retain the fibrous structure. For many purposes the quenching medium may be a sodium chloride brine, and if desired lime may be suspended in the brine.

Fused salt baths are desirable because when the article is removed it is coated with a film of the salt which protects it against scaling and decarburization during the forming operation. It also may act as a heat insulator, to minimize cooling prior to quenching. The addition of lime to the quenching bath is desirable because it minimizes the formation of vapor pockets and thus insures rapidity and uniformity of quenching.

After the article has been quenched it is removed from the dies, cleaned, and tempered to a hardness appropriate for its intended service.

As exemplifying the benefits which may be derived from the practice of the invention, reference may be made to tests in which there was used a silico-manganese spring steel containing 0.64 per cent of carbon, 0.89 per cent of manganese, 0.021 per cent of phosphorus, 2.2 per cent of silicon, and 0.023 per cent of sulfur. The steel was hot-rolled to produce round rod, such as is used in the manufacture of helical springs, having a diameter somewhat greater than  $\frac{3}{4}$  inch, the intended final diameter. The rod was then given a finishing pass at about 1200° F. to bring it to  $\frac{3}{4}$  inch diameter, thus producing the fibrous structure referred to hereinabove. The hot-sized rod was then cut to lengths which were immersed in a salt bath and heated to 1550° F. in two and one-half minutes, which time included the interval necessary to bring the rod to temperature and effect complete penetration of the heat. At the end of the interval stated the rod was removed and quenched. It was then tempered at 800° F. for one hour. The rod treated in this manner showed mechanical properties as follows, these being determined from test bars of standard shape and size:

| 60 | Strength, lbs./sq. in. |                    | Elongation, percent in two inches | Reduction of area, percent | Brinell hardness |
|----|------------------------|--------------------|-----------------------------------|----------------------------|------------------|
|    | Yield point            | Ultimate tensile   |                                   |                            |                  |
| 65 | 180,600<br>200,700     | 239,000<br>241,000 | 5.0<br>4.5                        | 18.0<br>15.2               | 477<br>514       |

The combination of properties represented by the foregoing tests is unusual and is highly desirable for spring steel purposes. The properties of the hot-sized material are presumably actually better than those given because in the preparation of the standard test bars used the outer portion of the bar, which is the most highly fibered, is removed. It follows that a spring made from

the hot-sized bar, without machining, would have still better properties.

As further exemplifying the practice of the invention, steels of similar composition were rolled to produce strip such as is used in making elliptical springs. These steels contained from 0.58 to 0.62 per cent of carbon, from 0.78 to 0.86 per cent of manganese, from 0.022 to 0.026 per cent of phosphorus, from 1.86 to 1.98 per cent of silicon, and from 0.025 to 0.029 per cent of sulfur. The ingots were hot-rolled to produce a flat whose sectional area was somewhat greater than that of the finished spring, and they were then brought to finished size by a hot-finishing pass at about 1200° F. The hot-sized strip was then cut into lengths for spring manufacture which were heat-treated in the same manner as in the foregoing example. Two of the bars, which were  $1\frac{1}{4}$  inches wide and  $\frac{3}{2}$  inch thick, showed ultimate tensile strengths of 229,000 psi and 284,480 psi. Other results were as follows:

| Size of flat                       | Yield point, lbs./sq. in. | Ultimate tensile, lbs./sq. in. | Elongation, percent in two inches | Reduction of area, percent | Brinell hardness | 25 |
|------------------------------------|---------------------------|--------------------------------|-----------------------------------|----------------------------|------------------|----|
| $1\frac{3}{4} \times \frac{1}{4}$  | 198,900                   | 206,189                        | 8.0                               | 11.7                       | 415              |    |
| $2 \times \frac{3}{16}$            | 175,760                   | 219,059                        | 8.5                               | 16.9                       | 415              |    |
| $2\frac{1}{4} \times \frac{1}{16}$ | 174,719                   | 195,720                        | 9.0                               | 9.1                        | 388              | 30 |

The foregoing tests exemplify the manner in which the hardening operation may suitably be conducted. It will be observed that in the specimens of the dimensions given the article was heated to 1500° F. in two and one-half minutes. It will be understood, however, that exact times of heating can not be given for all purposes because the time of heating will depend upon the composition of the steel, the section of the piece, and the treating temperature. As to composition, it is known to those skilled in the art that some steels are more resistant to the effect of heat treatment than others. For instance, the chromium steels generally tend to recrystallize somewhat sluggishly and where steels exhibit this property they may be exposed longer than others without danger of impairing the fibrous structure. Also, the section or mass of the piece will play its part, it being generally true that the greater the thickness the greater the time that will be required to bring the article to temperature. For the reasons stated it is not practical or possible to give precise heating times which will produce optimum results under all conditions and for the production of all combinations of properties, but generally speaking, as the time of heating is increased there is a tendency to destroy the fibrous structure which results from hot-working and hot-sizing, and due regard must be given to this factor. The criterion is that the heating period must be short enough and quenching carried out sufficiently rapidly that the fibrous structure is substantially retained. It may be said, however, that in the manufacture of springs a heating time of a few minutes, say two to three minutes, suffices.

Similarly, the temperature of heat treatment will vary according to the composition of the steel as is known to those skilled in the art.

Reference has been made to the use of fused salt baths for rapid heating of the article in the hardening step. The advantages of such heating media have been explained. It is possible, however, to heat in other manners, as in electric fur-

naces, or by other suitable heating means, particularly in the case of steels which recrystallize sluggishly. In general, it is desirable in such cases to heat the steel in an inert atmosphere.

Various modifications are, of course, permissible. Thus, although the invention has been exemplified by reference to silico-manganese spring steel, it is applicable generally to steels whether of the plain carbon or of the alloy variety. In both cases the carbon content, and in the latter instance the specific alloying elements and their amounts, will be selected according to service requirements. In any event, the application of the invention provides properties which exceed those of the same steel fabricated according to prior art procedures.

Also, in the foregoing tests reference has been made to hot-rolling but it will be understood that other types of hot-working are applicable, such as die-forging, hammering, and the like.

The precise degree of oversize of the stock prior to hot-sizing will depend in part upon the size of the final shape and the required properties. In sizing the fibrous structure is most pronounced at the surface if the stock is not reduced much in sectional area in hot-sizing it. The greater the reduction in the sizing step the more deeply will the fibrous structure penetrate, and based upon these factors the degree of oversize prior to hot-sizing is determinable. By reason of the location and character of stresses in springs, it may be said that for such purposes it is not necessary for the fibering to penetrate deeply into the bar.

Usually it will be desirable to de-scale the hot-sized shape prior to heat treatment.

In springs, whether helical, elliptical, or spiral, the major stresses are tension and compression in the longitudinal direction of the bar or rod. For instance, in a leaf spring the maximum stresses are tension and compression largely concentrated adjacent the upper and lower surfaces of the leaf. The fibrous structure of products made in accordance with this invention is particularly desirable for spring purposes because the grains are thus disposed in the direction of the major stresses, and through increased resistance to tension and true compression, coupled with reduction of shear and torsion stresses, improved life is assured.

The fibrous structure is further desirable in the case of helical springs because when the spring is put under tension or compression in use the coiled rod is subjected to torsional stresses normal to the direction of the fibers. As the metal undergoes torsional strain, a component of stress longitudinally of the bar is introduced as a result of the disposition of the fibers, which permits the helical spring to resist the compressive and torsional stresses to which it is subjected in use better than such springs made in accordance with prior practice in the art.

As noted hereinabove, the heat treatment is conducted to harden the article. This involves, generally, a change from one type of space lattice to another, and the reaction is more rapid than that involved in complete recrystallization, although recrystallization can not be wholly avoided. I believe that the incipient recrystallization is valuable, however, because the fibers are bonded thereby, improving strength. While I do not not confine myself to this theory, I believe also that such incipient equi-axing of the grains sets up internal stresses which are beneficial in that the service stresses, for instance in the case of

springs, must overcome this internal stress before their effect upon the spring in the direction of the service stress is encountered. In other words, the internal strain opposes the service stress which increases the safe imposed stress value of the part, or it withstands a greater elastic loading than a part not having the structure provided by the invention. 5

The same properties adapt the articles made in accordance with the invention to other uses 10 also, as will be understood in the art.

According to the provisions of the patent statutes, I have explained the principle and manner of practicing my invention, and have described what I now consider to be its best embodiment. 15 However, I desire to have it understood that, within the scope of the appended claims, the invention may be practiced otherwise than as specifically described.

I claim:

1. That method of treating steel which comprises hot-working a piece of steel to form oversized stock, then hot-sizing said stock at a temperature close to but below the recrystallization range of the steel, thereby producing a sized shape 25 having a fibrous structure extending inwardly a substantial depth from the surface, and heating such shape in the austenite range and quenching to harden it while substantially preserving said structure. 30

2. That method of treating steel which comprises hot-working a piece of steel to form oversized stock, then hot-sizing said stock at a temperature close to but below the recrystallization range of the steel, thereby producing a sized shape 35 having a structure of fibers elongated in the direction of working and extending inwardly a substantial depth from the surface, and heating such shape in the austenite range and quenching it with substantial avoidance of recrystallization. 40

3. That method of treating steel which comprises hot-working a piece of steel to form oversized stock, then hot-sizing said stock at a temperature close to but below the recrystallization range of the steel, to produce thereby a sized 45 shape having a fibrous structure of parallel elongate grains aligned with the longitudinal axis of the shape and extending inwardly a substantial depth from the surface, heating such shape rapidly to a temperature within the austenite range 50 for a period of time such that said structure is not substantially destroyed, and quenching the thus heated steel rapidly to preserve such structure.

4. That method of treating steel which comprises hot-working a piece of steel to form oversized stock, hot-sizing said stock at a temperature close to but below the recrystallization range to bring it to finished size, thereby producing a sized shape having a fibrous structure and extending inwardly a substantial depth from the surface, heating the sized shape rapidly to a temperature within the austenite range, and quenching the heated piece before said fibrous structure has been substantially changed. 55

5. That method of treating steel which comprises hot-working a piece of steel to form a shape close to but somewhat oversize, then bringing the shape to finished size by a hot-finishing pass at a temperature close to but below the 70 recrystallization range, to produce thereby a sized shape having a fibrous structure of elongate parallel grains extending inwardly a substantial depth from the surface, heating the sized shape rapidly to a temperature within the austenite 75

range for a period of time such that said fibrous structure is substantially preserved, and quenching the heated piece before such heating effects substantial recrystallization of such fibrous structure.

5 6. That method of treating steel which comprises hot-rolling a piece of silico-manganese spring steel to form oversized stock, hot-rolling said stock at a temperature of about 1200° F. to bring it to finished size, thereby producing a sized shape having a fibrous structure extending inwardly a substantial depth from the surface and composed of elongate grains parallel to the longitudinal axis of the shape, heating the sized shape rapidly to a temperature of about 1550° F., and quenching the heated piece before said fibrous structure has been substantially changed.

10 7. That method of making springs which comprises hot-working a piece of steel to form oversized bar or strip stock, then hot-sizing said stock at a temperature close to but below the recrystallization range of the steel, thereby producing a sized shape having a fibrous structure of elongate grains and extending inwardly a substantial depth from the surface, cutting said hot-sized stock to spring length, heating such length rapidly to a temperature within the austenite range for a period of time such that said structure is not substantially altered, shaping the spring 15 20 25 while so heated, and quenching the thus heated steel rapidly to preserve said fibrous structure.

20 8. That method of treating steel which comprises hot working a piece of steel to form oversized stock, hot sizing said stock at a temperature close to but below the recrystallization range 30 35 of the steel to bring it to finished size, thereby

producing a sized shape having a fibrous structure and extending inwardly a substantial depth from the surface, heating the sized shape to a temperature to convert the steel to the austenitic condition, and quenching when such condition has been produced but before equi-axing of the fibrous grains has occurred.

9. That method of treating steel which comprises hot working a piece of steel to form oversized stock, hot sizing said stock at a temperature close to but below the recrystallization range of the steel to bring it to finished size, thereby producing a sized shape having a fibrous structure and extending inwardly a substantial depth from the surface, heating the sized shape to a temperature to convert the steel to the austenitic condition, quenching when such condition has been produced but before equi-axing of the fibrous grains has occurred, and tempering after quenching to produce a troostitic-sorbitic structure in 15 20 25 the steel.

10. As a new article of manufacture, a hot-worked and heat-treated steel article made by hot working a piece of steel to form over-sized stock, hot sizing said stock at a temperature close to but below the recrystallization range to bring it to finished size thereby producing a sized shape having a fibrous structure composed of elongated substantially parallel grains substantially stable, on reheating, against grain growth due to residual working strain, and heating the sized shape rapidly to a temperature within the austenite range and quenching it before substantial recrystallization has taken place and thereby substantially preserving said structure.

30 35 WILLIAM J. MERTEN.